

Aug. 9, 1938.

F. H. DRIGGS ET AL

2,125,896

ARTICLE OF MANUFACTURE AND METHOD OF PRODUCING THE SAME

Filed July 10, 1934

2 Sheets-Sheet 1



1.



2.



3.



4.



INVENTOR  
F. H. DRIGGS  
H. W. HIGHRITER

BY *M. T. Reges*  
ATTORNEY

Aug. 9, 1938.

F. H. DRIGGS ET AL

2,125,896

ARTICLE OF MANUFACTURE AND METHOD OF PRODUCING THE SAME

Filed July 10, 1934 2 Sheets-Sheet 2

Fig. 5.



Fig. 6.



Fig. 8. Fig. 9.



INVENTOR  
F. H. DRIGGS  
H. W. HIGHRITER  
BY *M. T. Reges*  
ATTORNEY

Patented Aug. 9, 1938

2,125,896

# UNITED STATES PATENT OFFICE

2,125,896

## ARTICLE OF MANUFACTURE AND METHOD OF PRODUCING THE SAME

Frank H. Driggs, Highland Park, Ill., and Harry W. Highriter, Verona, N. J., assignors, by mesne assignments, to Westinghouse Electric and Manufacturing Company, East Pittsburgh, Pa., a corporation of Pennsylvania

Application July 10, 1934, Serial No. 734,450

15 Claims. (Cl. 256—35)

This invention relates to an improved article of manufacture and to a novel method for producing the same. In its more specific aspect the invention is directed to an improvement in anodes for X-ray tubes and to the method for producing the same.

An X-ray tube generally consists of an envelope containing an anode and a thermionic cathode therein. The cathode is incandescent for supplying electrons and when an appropriate potential is applied between these electrodes, the electrons emanating from the cathode are forced to the anode and bombard the target portion of the same to produce X-rays. During this bombarding action some of the energy possessed by the electrons is converted to heat energy at the anode. The anode may consist of a target composed of a refractory metal, generally tungsten, embedded in a backing of metal, such as copper, having high thermal and high electrical conductivity characteristics. In the course of X-ray tube operation, it is found that X-ray tubes sometimes fail because of anode fusion. In some cases serious cracking of the copper close to the target occurs. The cracking generally takes place along the grain boundaries approximately one grain diameter distant from the edge of the target. The cracking first takes place on the surface of the copper around the target and gradually increases in both amount and scope until it extends underneath the target as well. Thus there is formed an isolated zone of copper around the tungsten which is in poor thermal contact with the remainder of the copper backing. When this condition is reached the high temperature, which this copper in contact with the tungsten attains during operation, is sufficient to melt the copper thus causing a failure in the tube.

Probably the basic cause of this type of failure in the copper lies in the wide difference in thermal coefficients of expansion of tungsten and copper. At room temperature the coefficient of expansion of copper is about five times that of tungsten. During operation of the tube the entire anode is probably subjected to temperature changes varying from room temperature to about 500° C. It is our belief that the expansion and contraction of the tungsten and copper due to these temperature variations cause the cracking in the copper to take place.

It is in order to obviate this difficulty that this invention is primarily concerned. Briefly this disadvantage is removed by providing a reinforcement in the copper in the vicinity of the target to take up some of the stresses which would otherwise be taken up by the copper per se. That is, the reinforcing means which we provide in the copper adjacent the target reduces the stresses so that the stresses that are borne by the copper are less than those necessary to cause copper

cracking. In addition, the reinforcing means so distributes the stresses as to prevent the stresses from exceeding the tensile strength of the boundary between adjacent crystals.

An object of our invention is to provide an improved clad metal.

Another object of our invention is to provide an improved anode for an electric discharge device such as an X-ray tube.

A still further object of our invention is to provide a novel method for producing the same.

These and other objects of our invention will be readily understood from the following description and drawings wherein,

Figure 1 represents a fragmentary view partly in section of an X-ray anode embodying our invention, with the section taken along line I—I of Figure 2;

Figure 2 represents a plan view of an X-ray anode embodying our invention, with the embedded reinforcing elements shown by dotted lines;

Figure 3 represents a form employed and illustrates one of the steps of forming the reinforcing element;

Figure 4 is a perspective view only partially completed and showing the configuration of the reinforcing element;

Figure 5 represents the apparatus employed for carrying out one of the steps of our invention;

Figure 6 represents the product obtained after carrying out one step of our invention in the apparatus illustrated in Figure 5;

Figure 7 represents the apparatus employed in carrying out another step of our invention;

Figure 8 illustrates a modification of Figure 1 and embodying our invention; and

Figure 9 illustrates a further modification of Figure 1 and embodying our invention.

As illustrated in Figures 1 and 2, an improved anode embodying our invention comprises a copper rod 10 of high thermal and electric conductivity characteristics. The target end of the rod has an angular face at about twenty degrees to the longitudinal axis of said rod. Embedded in said rod and forming a portion of said angular face is a target 11 composed of tungsten or the like.

The width of the target 11 is about half that of said angular face and its length is about three-quarters that of said face. The target is so disposed with relation to said rod that its effective face is flush with the copper portion of said rod which, together define the angular face. The upper extremity of the target is flush with the upper extremity of said rod and the target is located midway between the sides of said face.

For the prevention of copper cracking in the copper adjacent the longitudinal and transverse edges of the target we provide a reinforcing means

12. The reinforcing means 12 may comprise a plurality of strands of refractory material of high tensile strength. The material may be composed of tungsten, molybdenum or the like whose melting point is higher than that of copper. Reinforcing means that we have found suitable for our purposes consists of a basket weave construction partially illustrated in Figure 4 and composed on tungsten wires that may be of 5, 10, or 17 mil. diameter. Although all three sizes of wires were equally good as reinforcing means, we found that the 10 mil. size was the most desirable from the standpoint of ease of handling and general stability of the winding after weaving the same.

15. As illustrated in Figures 1 and 2, the reinforcing element is so disposed that it is completely embedded in the copper with its lower transverse and its longitudinal sides being adjacent and opposite the corresponding sides of the target 11 so that a sufficient proportion of the individual turns of the wire shall be embedded in those copper crystals immediately adjacent the target and also in crystals located a grain diameter from the first group of crystals.

20. 25. The upper transverse side of said reinforcing element is located near the corresponding side of the target but adjacent the lower face of the target. The reinforcing element thus being embedded in at least the first two adjacent rows of crystals, extends through the boundary between these rows closest to the sides of the target and takes up the stresses which might otherwise be borne by the crystals. Because of the high tensile strength of the reinforcing wires, there is no cracking of the copper, even when the target is subjected to higher bombardment than is customary with present type anodes.

30. 35. The reinforcing means need not be confined only to the position shown in Figure 1. Besides employing only one reinforcing element located adjacent the transverse and longitudinal sides of the target, we may also employ another reinforcing element 13 in conjunction therewith, as shown in Figure 8. The other reinforcing element 13 consists of a mat of fine tungsten wire embedded in the copper backing adjacent the lower face of the target 11, with some portions thereof being embedded in that group of copper crystals immediately adjacent the bottom of the target 11 and the rest of it being distributed throughout a large proportion and if desired all of the copper behind the target. As a matter of fact we may employ a mat of tungsten wire which may completely surround the target that is embedded in the copper.

40. 45. 50. 55. Even in those tubes which employ targets that cover the entire upper face of the copper, cracking appears in that portion of the copper adjacent the bottom of said target. To eliminate this objectionable feature, an annulus 14 is composed of a number of turns of fine tungsten wires which may have their separate turns distorted along their lengths. The annulus is embedded in the copper just below the target and near the outer periphery of the copper backing.

60. 65. 70. 75. Although our improved X-ray anodes above described may be produced by following any particular series of steps that is found convenient, we have employed the following method with good success. A cylindrical solid graphite element 20 having a portion thereof cut away and being complementary to the configuration of the upper end of the anode to be produced is placed in a carbon crucible 21. The angular face of the element 20 has a target 11 located thereon and

held thereto by means of small tungsten wires 22 that are embedded in the carbon form and bent over that face of the tungsten target 11 which is to be coated.

5. 10. 15. The lower transverse end of the target 11 rests against the shoulder of the carbon form and the longitudinal sides of the target 11 are located inwardly from the sides of the form with the upper transverse end of the target located below the upper edge of the form. The reinforcing element 12 is also secured to the block, with the lower transverse side resting upon the shoulder of the form and being contiguous with that end of the face of the target to be coated, the longitudinal and transverse sides of the reinforcing element 12 extending along and being contiguous with the corresponding sides of the target 11.

20. 25. 30. 35. Our invention contemplates the employment of any type of reinforcement. We have found that good results are obtained by forming a reinforcing element of basket weave design. This may be produced by employing a forming element 25 having a plurality of rows of spaced posts defining the length and breadth of the weave to be produced. A wire of tungsten about 10 mils. in diameter is wound as shown in Figure 3 to produce the element shown in Figure 4. After the weave is wound around the posts, it may be permanently set by suitable heat treatment in a hydrogen furnace. The weave 12 is removed from the supporting posts and ready to be secured to the block 20. The reinforcement 12 is also held in place by tungsten wires 22 embedded in the carbon form. The carbon element 20 having the target 11 and the reinforcing means 12 affixed thereto may be treated in a hydrogen furnace so that their surfaces shall be absolutely oxygen free.

40. 45. 50. 55. 60. 65. 70. 75. The button 11 and reinforcement 12 may, if desired, be so treated before mounting on the carbon form. In either case the target and reinforcing element are subject to hydrogen treatment at about 1500 degrees centigrade for about an hour. Added to the crucible containing the form 20 to which are affixed the button 11 and reinforcement 12 is a short rod of copper 24. The crucible and its contents are placed in a hydrogen furnace 23 and the same are heated in any convenient manner in order to fuse the copper. This heating is carried out with pure hydrogen passing through the furnace. The hydrogen keeps the readily oxidizable tungsten free from oxidized patches or particles and also reduces any small quantity of oxygen contained in the copper. The copper becomes molten during this heat treatment and flows around and wets the tungsten. The hydrogen flow and heating are maintained for any desired length of time. Thereafter the crucible and its contents are allowed to cool.

80. 85. 90. 95. Instead of performing the hydrogen treatment of the target and the coating as separate and distinct operations, we may accomplish both results in a single operation. For these purposes the form 20, the target 11 and the reinforcing element assembled as shown in Figure 5 may be placed in an open boat with the target face to be coated uppermost. A mass of "pure" copper shavings is placed on that face to be coated. This group of elements is inserted in a hydrogen furnace where they are heated in the presence of a stream of pure hydrogen which cleans the target by reducing any oxide present thereon. The copper fuses and flows onto the target and reinforcing element and wets the same.

In this heating step, as in the first fusion step heretofore set forth, the copper is maintained at or above its fusion temperature and in the presence of pure hydrogen for such a length of time that the tungsten button and the tungsten reinforcing element may be completely wetted by the copper. The presence of hydrogen at the temperature of copper fusion reduces any copper or tungsten oxides that may have been present. Thus a good bond between the copper and the target 11 and reenforcing element is obtained, with the copper extending about one-sixteenth of an inch and preferably of less thickness than that required for the production of a copper coating having a honeycomb structure due to large hydrogen absorption. This slug is subjected to the same subsequent operations as is the slug 26 hereinafter identified.

The slug 26, as shown in Figure 6 and consisting of the carbon form, the target 11, reinforcing element 12 and the copper 24 is removed from said crucible and placed in a longer crucible 27. The crucible 27, together with its contents, is placed in a long furnace. Inserted in said crucible 25 is also a volume of copper 28 that is large as compared with the volume of copper 24.

Either pure nitrogen or an admixture of 90 percent nitrogen and 10 percent hydrogen is continually passed through this furnace which is heated to fuse the copper. The entire mass of copper is rendered molten and then allowed to cool. The bar which consists of the carbon form 20, the button 11, reinforcing element 12 and a single copper backing is withdrawn from the furnace and the carbon backing is detached from the rod leaving our X-ray anode which is then cleaned and polished.

Although our invention has been described with some particularity it is to be limited only by the prior art because it is susceptible to numerous modifications, some of which we ourselves have illustrated and briefly described.

What is claimed:

1. An anode for an X-ray tube comprising a composite unit including a plurality of metallic constituents of different compositions and having different coefficients of linear expansion, said constituent whose coefficient of linear expansion is the lower having a high melting point, filamentary means separate from the remaining metallic constituents and totally imbedded in said constituent whose coefficient of linear expansion is the higher for reducing the tendency of said last named constituent to cracking upon repeatedly raising and lowering the temperatures of said constituents, and without affecting the thermal conductivity between said constituents, the fusion point of said filamentary means being higher than that of said constituent whose coefficient of linear expansion is the higher, said filamentary means being disposed immediately adjacent the surface of contact between said metallic constituents.

2. An X-ray anode comprising a composite unit including a plurality of metallic constituents, one of said constituents being composed of a refractory metal and another of said constituents composed of a metal whose melting point is much lower than that of said refractory metal, the coefficients of linear expansion of said constituents being different, filamentary means separate from the remaining metallic constituents and totally imbedded in said metal of lower melting point for reducing the tendency of said metal of lower melting point to cracking upon repeat-

edly raising and lowering the temperatures of the same, and without affecting the thermal conductivity between said constituents, said filamentary means being distorted along its length and having portions thereof located entirely within the boundaries of said metal of lower melting point, and being disposed immediately adjacent the surface of contact between said metallic constituents.

3. An electrode for an electric discharge device comprising a body of refractory metal and a body of metal having high heat and electrical conductivity characteristics, said bodies being contiguously joined together, and means separated from said refractory metal body and totally imbedded in said second mentioned body forming a layer having an average coefficient of linear expansion intermediate that of the two bodies to take up some of the stresses which would otherwise be borne by said second mentioned body to reduce the tendency of said second mentioned body to cracking, without affecting the thermal conductivity between said bodies, said means being located adjacent the surface of contact between said bodies.

4. An electrode for an electric discharge device comprising a body of refractory metal and a body of metal having high heat and electrical conductivity characteristics contiguously joined together, and filamentary means separate from said refractory metal body and totally imbedded in that zone of said second mentioned body which normally cracks upon repeatedly raising and lowering the temperatures of said bodies to form a layer having an average coefficient of linear expansion intermediate that of the two bodies, said means reducing the tendency of said second mentioned body to cracking at that zone upon said temperatures taking place, without affecting the thermal conductivity between said bodies, said zone being adjacent the surface of contact between said bodies.

5. An X-ray anode comprising a target joined to a body of metal of high heat and electrical conductivity characteristics, and means separate from said target for taking up some of the stresses that otherwise would be borne by said body and forming a layer having an average coefficient of linear expansion intermediate said target and body to reduce the tendency of said body to cracking upon repeatedly raising and lowering the temperatures of said target and body, without affecting the thermal conductivity between said target and body, said means being totally disposed in said body adjacent the contacting surface between said body and target.

6. An X-ray anode comprising a body of refractory metal and a body of metal having high heat and electrical conductivity characteristics joined together, and means separate from said refractory metal body for reducing the tendency of said second mentioned body to cracking, without affecting the thermal conductivity between said bodies, said means being totally imbedded in said second mentioned body to form a layer having an average coefficient of linear expansion intermediate that of the two bodies, with portions of said means being imbedded in the crystals of said second mentioned body closest to said first mentioned body and also in those crystals of said second mentioned body immediately adjacent said first mentioned crystals.

7. An X-ray anode comprising a body of refractory metal and a body of metal having high heat and electrical conductivity characteristics

- joined together, and reinforcing means separate from said refractory metal body totally imbedded in that zone of said second mentioned body which otherwise would crack and forming a layer having an average coefficient of linear expansion intermediate that of the two bodies to reduce the tendency of said cracking at that zone upon raising and lowering the temperatures of said bodies, and without affecting the thermal conductivity between said bodies, said zone being located adjacent the contacting surface of said bodies.
8. An X-ray anode comprising a target, a body of metal having high heat and electrical conductivity characteristics, said target and body being contiguously joined together, and filamentary means separated from said target and totally imbedded in said body to form a layer having a coefficient of linear expansion intermediate that of the two bodies for reducing the tendency of said body to cracking upon repeatedly raising and lowering the temperatures of said target and body, without affecting the thermal conductivity therebetween, said means having portions thereof imbedded in the crystals of said body immediately adjacent said target and in the crystals of said body adjacent said first mentioned crystals.
9. An article of manufacture comprising a composite unit including a plurality of metallic constituents of different compositions and having different coefficients of linear expansion, one of said constituents composed of a metal whose melting point is lower than that of said refractory metal, and filamentary means imbedded in said metallic constituent of lower melting point for reducing the tendency of said lower melting point metal to cracking upon repeatedly raising and lowering the temperature of said constituents, said filamentary means being of zig-zag design along a portion of its length, the melting point of said filamentary means being higher than that of said metal of lower melting point.
10. An article of manufacture comprising a composite unit including a plurality of metallic constituents of different compositions and having different coefficients of linear expansion, one of said constituents being composed of a refractory metal and another of said constituents being composed of a metal whose melting point is materially lower than that of said refractory metal, a filamentary means simulating a basket weave imbedded in said metal of lower melting point to reduce the tendency of the same to cracking, said means composed of a substance whose melting point is higher than that of said metal of lower melting point.
11. An article of manufacture comprising a refractory metallic body, another metallic body of lower melting point, said second body being joined to and in contact with said first mentioned body, and a reinforcing means imbedded in said second metallic body to form a layer having a coefficient of linear expansion intermediate that of the two bodies for reducing the tendency of said second metallic body to cracking upon repeatedly raising and lowering the temperatures of said bodies, the fusion point of said means being greater than that of said second body, said reinforcing means being disposed immediately adjacent the surface of contact between said bodies
- without affecting the thermal conductivity between said bodies.
12. An article of manufacture comprising a button composed of a refractory metal body and a body having high heat and electrical conductivity characteristics, said bodies being joined together, and means separate from said metal body imbedded in said second mentioned body and forming a layer having a coefficient of linear expansion intermediate that of the two bodies located adjacent the contacting surface of said bodies without affecting the thermal conductivity therebetween for reducing the tendency of said second mentioned body to cracking, said means having a tensile strength which exceeds that of said second mentioned body.
13. An X-ray anode comprising a target and a body of metal of high thermal and electrical conductivity characteristics joined together, the coefficients of linear expansion of said target and body being different, and means adjacent the surface of said contact between said target and body and separated therefrom and being imbedded in said body without affecting the thermal conductivity between said body and said target for reducing the tendency of said body to cracking upon repeatedly raising and lowering the temperature of said target and body, said means composed of a substance whose tensile strength is greater than that of said body, said means having a melting point which is higher than that of said body.
14. An X-ray anode comprising a target and a body of metal having good thermal and electrical conductivity characteristics joined together, the coefficients of linear expansion of said target and body being different, filamentary means adjacent said target and separated therefrom and imbedded in that zone of said body which is subjected to high stresses without affecting the thermal conductivity between said target and said body, said means composed of a substance having a higher tensile strength than that of said body and also having a higher melting point than that of said body, said means adapted to take up some of the stresses at that zone which might otherwise be borne by said body and thus to reduce the tendency of said body to cracking upon repeatedly raising and lowering the temperature of said target and body, said zone being located adjacent the surface of contact between said target and body.
15. An X-ray anode comprising a target, a body of metal having high heat and electrical conductivity characteristics, said target and body being contiguously joined together, and filamentary means separated from said target imbedded in said body and forming a layer having a coefficient of linear expansion intermediate that of said target and said body located adjacent the surface of contact between said target and body without affecting the thermal conductivity therebetween for reducing the tendency of said body to cracking upon repeatedly raising and lowering the temperatures of said target and body, said means composed of a substance having a higher melting point and a higher tensile strength than does said body.

FRANK H. DRIGGS.  
HARRY W. HIGRITER.